# EUROPEAN PATENT SPECIFICATION

(11) **EP 2 161 349 B1**
(45) Date of publication and mention of the grant of the patent: **17.10.2018**
(21) Application number: 09008026.8
(22) Date of filing: 19.06.2009
(51) Int. Cl.: C22C 9/05, C22F 1/08

(54) **METHOD FOR PRODUCING A COPPER-BASED WHITE ALLOY FOR PRODUCING NATURALLY ANTIBACTERIAL ARTICLES**
VERFAHREN ZUR HERSTELLUNG EINER WEISSMETALLLEGIERUNG AUF KUPFERBASIS ZUR HERSTELLUNG VON NATÜRLICHERWEISE ANTIBAKTERIELLEN ARTIKELN
PROCEDE DE PRODUCTION D'ALLIAGE BLANC A BASE DE CUIVRE POUR PRODUIRE DES ARTICLES NATURELLEMENT ANTIBACTERIENS

(30) Priority: 01.09.2008 IT TO20080649
(43) Date of publication of application: 10.03.2010
(73) Proprietor: KME Italy S.p.A., 50127 Firenze (IT)
(72) Inventor: Ammannati, Niccolò, 55051 Fornaci di Barga (IT); Martellucci, Elena, 55051 Fornaci di Barga (IT); Giusti, Aldo, 55028 Piano di Coreglia (IT); Sbrana, Armando, 50100 Lucca (IT)
(74) Representative: Griepenstroh, Jörg

(56) References cited:
- EP-A- 1 880 776
- WO-A-00/68447
- CA-A1- 964 408
- DE-B- 1 224 937
- JP-A- 60 072 695
- US-A- 3 725 052
- US-A- 5 725 682
- MUKHERJEE, D. ET AL: "Antifouling properties of copper-manganese alloys" TOOL & ALLOY STEELS , 27(9), 287-9 CODEN: TASTDL; ISSN: 0377-9408, 1993, XP009122240
- MUKHERJEE, D. ET AL: "SRB-cidal properties of some copper-manganese alloys" BULLETIN OF ELECTROCHEMISTRY , 6(5), 499-500 CODEN: BUELE6; ISSN: 0256-1654, 1990, XP009122239
- MUKHERJEE, D. ET AL: "Corrosion resistant and antifouling behavior of Cu-Mn alloys in sea-water" BULLETIN OF ELECTROCHEMISTRY , 9(8-10), 427-9 CODEN: BUELE6; ISSN: 0256-1654, 1993, XP009122244

## Description

### Field of the art

The present invention relates to a method for producing articles made of a copper-based white alloy, wherein these articles are naturally antibacterial and simultaneously have an excellent mechanical resistance, an easy machinability, a high cleaning ease and an appearance similar to that of stainless steel.

### State of the art

It has been known since ancient times (ancient Egypt) that copper has disinfectant properties. More recently, copper and its alloys (brasses) have been investigated for their bactericidal properties on some pathogen microorganisms [H. T. Michels, ASTM Standardization NEWS, October 2006, pp. 29-31] and compared to stainless steel, on the surface of which the same pathogens that manage to survive on copper and alloys thereof only for a few hours, can instead survive30 days or more, in the absence of disinfectant treatment. US-EP approved antimicrobial abilities of tests have shown the copper and brasses against Staphylococcusaureus, Enterobacteraerogenes, E. Coli 0157:H7, Pseudomonas aeruginosa and MRSA (methicillin resistant Stafilococcus aureus).

However, copper and brasses have aesthetical and technological features which are generally considered inappropriate to validly replace stainless steel, for instance in the manufacturing of articles such as sanitaryware, sinks, tables, working surfaces for canteens or laboratories, basins for sanitary use, lockers, both because the mechanical features are typically much poorer than those of stainless steel, and because they are not white, but are instead of different colours such as red, pink and yellow. For all of these reasons, the use of copper and alloys thereof in the health field has been for the time being limited to components intended to remain hidden, for instance those of hydraulic or conditioning systems, such as finned heat exchangers.

There are also known, for producing jewels having an appearance similar to silver and for producing accessories for clothes, such as buttons and zips, white copper alloys, such as copper and nickel alloys, which however are nowadays increasingly less used due to the allergising effects of nickel, and the so-called "white brasses" , which are alloys of copper and zinc with the addition of manganese and/or aluminium, which have progressively replaced the previous, such as for instance the alloys disclosed in EP1306453B1 or in US6863746B, in the latter case the disclosed alloy being used to perform weldings on articles made of white gold. Although manganese may have a whitening effect on copper similar to that of nickel, the only known white alloys which do not contain nickel and are not brasses, are the so-called "manganins", used for manufacturing electrical resistors due to the low conductivity manganese imparts alloyed copper, already from a few percentage points.

MUKHERJEE, D. ET AL: "Antifouling properties of copper-manganese alloys" TOOL & ALLOY STEELS, 27(9), 287-9 refers an examination of corrosion resistant and antifouling properties of Cu-Mn alloys. It was seen that a right proportion of manganese as well as the inclusion of a rear earth and some exotic material may result in the lowering of corrosion, and at the same time in the liberation of an optimum amount of toxic ion to behave as an anti-fouling agent. The examined alloys have a Cu-Mn-combination of 70:30. The examples comprise Zn and Al. The authors conclude this paper after recording the fact that Ce and Ce-Ga modified CuMn alloys, depend on their medium and environment, which controls their selective properties and their better resistance, as far as corrosion and fouling resistance are concerned. MUKHERJEE, D. ET AL: "SRB-cidal properties of some copper-manganese alloys" BULLETIN OF ELECTROCHEMISTRY, 6(5), 499-500 refers to different copper-manganese alloys that have been fabricated and tested for their antifouling properties in SRB-cultures under static condition. Among the alloys experimented, the Cu-Mn alloy containing misch metal and gallium, besides being excellent antifoulant, acts as an efficient SRB-cide as well. The examined alloys were of the type 70:30 Cu-Mn.

A further paper dealing with the behavior of Cu-Mn alloys in sea-water is MUKHERJEE, D. ET AL: "Corrosion resistant 5-7, 9-15 and antifouling behavior of Cu-Mn alloys in sea-water" BULLETIN OF ELECTROCHEMISTRY, 9(8-10), 427-9. The authors conclude this study by highlighting the aspect of dual mechanism, observed in some alloyed and modified variety of Cu-Mn system, where the dissolution of toxic ions is probably assisted by the formation of an adherent oxide toxic-film, repelling the formation of the initial slime-layer.

CA 964 408 A1 discloses a method comprising casting a plate based on a Cu-alloy and comprising 30% Mn. A hot rolling from three inches to 0.35 inch is performed followed by cold rolling from 0.35 to 0.1 inch. It follows an annealing procedure for 1 h at 600 - 750°C for recrystallization.

DE 1 224 937 B refers to the use of copper alloys. The disclosed copper alloys may be used for bearings according to their friction properties. The alloy contains up to 8% aluminum, up to 5% Ni and up to 45% Zn. Further the alloy contains Tellur, Silicium and up to 12% Mangan. The alloy may be subject of hot forming or cold forming and annealing between 200 and 700°C for recrystallization. This document does not deal with articles that have antibacterial properties.

WO 00/68447 A discloses a copper alloy with a golden visual appearance. The material has a transverse electrical conductivities substantially similar to that of copper alloy C713 and when clad to a copper alloy C110 core, a transverse electrical conductivities substantially similar to both sides of a Susan-B.-Anthony-US-Dollar coin. The copper base alloy is a copper-manganese-zink-nickel alloy consisting for example by weight of 10-15% Zn, 7-12% Mn, 2-6% Ni or 10-14% Zn, 5-10% Mn, 2-6% Ni, optionally controlled contents of Cr, Al, Fe, P, the balance being Cu with inevitable impurities. Once a planchet is stamped from the clad material, the planchet is annealed prior to coining. The suitable annealing profile is 700°C for 15-20 minutes in an atmosphere of 96% by volume, of nitrogen and 4%, by volume, of hydrogen or other combustible gas mixtures. The copper alloys were hot rolled to a thickness of 0.5 inch, milled to remove oxides and then cold rolled to 0.03 inch and buffed to provide a constant surface finish. A copper alloy treated by this method has a golden visual appearance.

It is an object of the present invention to therefore allow the replacement of stainless steel for producing articles intended to be employed in the health and/or food field or for which the intrinsic antibacterial properties are in any case important, with a material that has an appearance similar to that of stainless steel, has a low tendency to get dirty, may easily be cleaned with common cleaning products and, especially, has intrinsic antibacterial features, so as not to require frequent disinfection operations which are required instead by stainless steel when used in health and/or food applications.

It is also an object of the invention to provide a method for producing articles, in particular intended to be employed in the health and/or food field, which are naturally, i.e. intrinsically, provided with antibacterial abilities, so as not to require frequent disinfections of the exposed surfaces.

### Summary of the invention

The invention relates to the method of claim 1 for producing articles, these articles being in particular intended to be employed in the health and/or food field, these articles being provided with intrinsic antibacterial properties.

In particular, the manganese, and possible other alloying elements, except for impurities, are present in an amount such as to determine machinability, colour and surface properties of the alloy similar to those of stainless steel and simultaneously intrinsic antibacterial properties of the articles on respective exposed surfaces thereof.

According to the invention, the employed alloy does not contain aluminium, except as an impurity and neither zinc nor other alloying elements, but exclusively manganese and copper. Tin, in case it is required, may also be contained as further alloying element, but again in very low percentages, preferably below 2% so as not to produce in use the segregation of precipitates or low-melting phases which impart fragility to the alloy.

In the preferred embodiment, said alloy exclusively contains, except for impurities, copper and manganese, copper being prevailing.

The content of manganese ranges, in any case, in varying percentages between 15% and up to 40% by weight and preferably in an amount such as to obtain a crystalline structure of the alloy, exclusively in alpha phase, at ambient temperature. The optimal nominal composition of the alloy according to the use of the invention is 80% copper and 20% manganese.

The composition of the alloy according to the use of the invention is in any case such as to display on the surface antibacterial properties directed at least against microorganisms selected from the group consisting of: E.coli, MSRA, Listeria monocytogenes.

In particular, the method of the invention comprises the steps of:
- casting a plate or a cylindrical ingot made of a copper-based alloy containing manganese as the main alloying element, in an amount such as to make the alloy white in colour and to impart a crystalline structure in alpha phase at ambient temperature thereto;
- subjecting the plate or ingot to a series of hot plastic deformation machining treatments in sequence (rolling or drawing or extrusion), to obtain a first, predetermined percentage of sectional reduction;
- subjecting the hot semifinished article to a series of cold plastic deformation machining treatments in sequence (rolling or drawing), to obtain a second, predetermined percentage of sectional reduction;
- subjecting the cold semifinished article thus obtained to one or more heat annealing treatments of complete re-crystallization, in a reducing atmosphere;
- subjecting the hot and/or cold semifinished article to at least one step of removing a surface layer thereof with a low manganese contents; and
- obtaining a desired article with the cold annealed semifinished article.

The alloy contains manganese in a varying weight percentage between 15% and 40% and does not contain aluminium, and preferably neither zinc, except as impurities.

Furthermore, the first and second predetermined percentages of sectional reduction are on the order of 90% and the step of complete re-crystallization annealing of the cold semifinished article is performed at a temperature ranging between 550°C and 750°C and for about 4 hours, if performed in a static furnace or for a total time of about 45 minutes, if performed in a tunnel type furnace.

A step of abrasive brushing is performed so as to remove a surface layer of the cold annealed semifinished article having a thickness of about 4 microns.

Thereby, complex articles such as sinks, basins,tanks, plates, working surfaces of bathroom details,as tables, furniture tops, well as tubes, bars or wires, for instance to produce handrails, handles, knobs, sieves, may be obtained according to the invention and substantially without virtually any scraps, the articles having the appearance of stainless steel and being provided at the same time with very good natural or intrinsic antibacterial properties, which substantially make common sterilisation operations with disinfectants useless or at least redundant. Similar stainless steel articles are usually subjected to these disinfection operations, by the way with results which are always less effective as many bacterial strains have developed a considerable resistance to commonly used disinfectants and to antibiotics and have therefore become a continuous danger, in particular in a hospital environment, such as MRSA or E- coli O157:H7.

Furthermore, according to the results of the experiments performed by the Applicant, the antibacterial properties of copper alloys experimentally tested on many different bacterial strains, are probably due to the surface migration, and therefore on the exposed surfaces of articles made with these alloys, of copper atoms, a migration that is interrupted by the presence of aluminium in the alloy.

Therefore, according to the invention, the presence of aluminium in the alloy, unless the latter is present only as an impurity (the presence of impurities is in any case inevitable) must be avoided.

### Brief description of the figures

A preferred embodiment of the invention will now be disclosed by way of mere non-limitative example with reference to the figures of the attached drawings, wherein:
- figure 1 shows a diagram that compares the mechanical properties of the alloy according to the invention with another copper alloy and with a stainless steel; and
- figures 2 to 4 comparatively show the biological properties of some copper alloys, among which the alloy of the invention, and of stainless steel, for different types of germs.

### Detailed description

Further features of the invention will be apparent from the following examples for carrying out the invention.

### EXAMPLE 1

Two 900 kg plates were prepared by casting, the plates having dimensions 1800 x 500 x 115 mm (length x width x thickness) and each having the mean composition shown in Table 1.

**Table 1**

| | Mean chemical composition | | | | | |
|---|---|---|---|---|---|---|
| Melting N. | Cu % | Mn % | Fe % | Ni % | Sn % | Pb % |
| P 88500 | 81.2 | 18.8 | 0.015 | 0.03 | <0.01 | 0.01 |
| P 88501 | 80.0 | 20.0 | 0.02 | 0.035 | <0.01 | 0.01 |

Plate P88501 was then used, due to its better quality (chemical composition identical to the nominal composition - 80% copper and 20% manganese).

The plate was subjected to a hot rolling process bringing it to 740°C for 3.5 hours and was subsequently rolled thus obtaining in subsequent steps a reduction in the section of about 90%; the thickness was in particular reduced from 115 mm to 10 mm in 8 steps, thus reaching a final temperature of about 660-670°; the hot-rolled product was cooled down to about 350°C before forcedly cooling down to ambient temperature with water.

The rolled product was then examined and analysed to detect the depth and nature of the surface layers oxidised and depleted of alloying elements (manganese).

The results which were obtained are shown in tables 2 and 3, which follow.

**Table 2**

| Thickness of the oxidising layers measured on both sides of the longitudinal section of Cu80Mn20 hot-rolled plate | | | | |
|---|---|---|---|---|
| Top - edge 1 | | | | |
| | Mean | MAX. m | MIN. m | ST.DEV. m |
| Side A | 25.48 | 73.71 | 3.98 | 18.65 |
| Side B | 24.28 | 47.81 | 10.76 | 9.09 |
| | | | | |

| Top - centre | | | | |
|---|---|---|---|---|
| | Mean | MAX. m | MIN. m | ST.DEV. m |
| SIDE A | 13.14 | 27.52 | 4.42 | 6.4 |
| SIDE B | 17.23 | 85.79 | 3.98 | 17.7 |
| | | | | |

| Top - edge 2 | | | | |
|---|---|---|---|---|
| | Mean m | MAX. m | MIN. m | ST.DEV. m |
| Side A | 13.26 | 28.73 | 6.78 | 6.07 |
| Side B | 37.75 | 100 | 5.18 | 27.46 |
| | | | | |
| | | | | |

| Bottom - edge 1 | | | | |
|---|---|---|---|---|
| | Mean m | MAX. m | MIN. m | ST.DEV .m |
| Side A | 20.81 | 41.04 | 5.98 | 9.82 |
| Side B | 17.42 | 35.48 | 6.77 | 7.39 |
| | | | | |

| Bottom - centre | | | | |
|---|---|---|---|---|
| | Mean m | MAX. m | MIN. m | ST.DEV .m |
| Side A | 17.92 | 39.06 | 9.57 | 6.51 |
| Side B | 5.45 | 12.9 | 3.59 | 2.26 |
| | | | | |

| Bottom - edge 2 | | | | |
|---|---|---|---|---|
| | Mean m | MAX. m | MIN. m | ST.DEV .m |
| Side A | 16.91 | 28.68 | 7.17 | 6.58 |
| Side B | 39.33 | 110.05 | 9.38 | 29.61 |

**Table 3**

| Chemical composition along a linear profile (from the outer surface to 17.5 microns deep) | | | | | | | | |
|---|---|---|---|---|---|---|---|---|
| Position | Top | | | | Bottom | | | |
| | Edge | | Centre | | Edge | | Centre | |
| | Wt% Mn | wt% Cu | wt% Mn | wt% Cu | wt% mn | wt% Cu | wt% Mn | wt% Cu |
| 0 | 30 | 70 | 58 | 42 | 21.7 | 78.3 | 44.3 | 55.7 |
| 1.75 | 12.1 | 87.9 | 10.7 | 89.3 | 0.5 | 99.5 | 8.6 | 91.4 |
| 3.5 | 18.8 | 81.2 | 19.9 | 80.1 | 12.3 | 87.7 | 17.1 | 82.9 |
| 5.25 | 20.5 | 79.5 | 20.4 | 79.6 | 18.2 | 81.8 | 19.6 | 80.4 |
| 7 | 20.7 | 79.3 | 20.5 | 79.5 | 19.8 | 80.2 | 20.5 | 79.5 |
| 8.75 | 20.3 | 79.7 | 20.1 | 79.9 | 20.2 | 79.8 | 20.8 | 79.2 |
| 10.5 | 20.3 | 79.7 | 23.6 | 76.4 | 20.4 | 79.6 | 20.4 | 79.6 |
| 12.25 | 20 | 80 | 20.2 | 79.8 | 21 | 79 | 20.4 | 79.6 |
| 14 | 20.1 | 79.9 | 19.9 | 80.1 | 21 | 79 | 20.7 | 79.3 |
| 15.75 | 19.3 | 80.7 | 19.9 | 80.1 | 21.2 | 78.8 | 19.9 | 80.1 |
| 17.5 | 19.5 | 80.5 | 20.2 | 79.8 | 21 | 79 | 20 | 80 |

As may be appreciated, the depth of the detected layers of oxidation and depletion of Mn were relatively high and discontinuous, but such that said layers could easily and totally be removed by the normal milling/scalping operations which are generally performed after hot-rolling.

Subsequently, the hot-rolled product, after the milling/scalping operation and subsequent removal of the oxidised layers and with depletion of manganese, was subjected to a cold-rolling operation, again obtaining a reduction in the section of about 90% (from 10 to 0.7 mm of thickness) in subsequent steps, with the consequent work hardening and increase of hardness. The cold-rolled product was then subjected to a heat annealing treatment in a static furnace in a reducing atmosphere at 600°C for 4 hours for the re-crystallization. This treatment has been selected on the basis of a series of laboratory tests at different temperatures, in order to identify the optimal treatment, as shown in table 4.

**Table 4**

| Structure and size of the grain of Cu80Mn20 samples after one hour of heat treatment at increasing temperatures. | | |
|---|---|---|
| | Mean size of the grain (mm) | |
| Heat treatment | 1 mm thickness | 0.5 mm thickness |
| 400 °C / 1 hour | Fibrous structure | Fibrous structure |
| 450 °C / 1 hour | Fibrous structure | Fibrous structure |
| 500 °C / 1 hour | Re-crystallization start | Re-crystallization start |
| 550 °C / 1 hour | 0.005 | 0.0075 |
| 600°C / 1 hour | 0.0075 | 0.0075 |
| 650 °C / 1 hour | 0.010 | 0.015 |

Test specimens of the rolled material were subjected to the common tests for identifying the mechanical properties, in comparison to reference materials (other copper alloys and stainless steel). The results which were obtained are shown in figure 1, where the hardness curves of the different materials are shown as a function of the strain hardening, and in the following tables.

**Table 5**

| Material | HV | E (GPa) | Rp(0,2) (MPa) | Rm (MPa) | A50mm (%) |
|---|---|---|---|---|---|
| CuMn20 | 119 | 118 | 260 | 470 | 32 |
| CuZn20 | 77 | 110 | 115 | 330 | 47 |
| AISI 304-316 | 129 | 193 | 205 | 515 | 40 |
| Tab.2 Comparison between different materials | | | | | |

**Table 6**

| Material | IE (mm) | IB | R (%) | H (%) | L.D.R. |
|---|---|---|---|---|---|
| CuMn20 | 10,6 | 70 | ≅100 | 4.9 | 2,12 |
| CuZn20 | 10,6-12 | 66-68 | ≅96-100 | - | 1,94-2,00 |
| AISI 304-316 | 11-12 | - | ≅50-60* | - | 2,18-2,25* |
| Tab.3 Formability properties | | | | | |

**Table 7**

| | **Cu80Mn20** | | **Cu80Zn20** | | **Aisi 304** | |
|---|---|---|---|---|---|---|
| temper | Rp (Mpa) | Rm (Mpa) | Rp (Mpa) | Rm (Mpa) | Rp (Mpa) | Rm (Mpa) |
| **Annealed** | **256** | **493** | **115** | **330** | **205** | **515** |
| **1/4 Hard** | **308** | **498** | **300** | **420** | **413** | **690** |
| **1/2 Hard** | **564** | **597** | **440** | **510** | **606** | **827** |
| **Hard** | **820** | **860** | **480** | **570** | **772** | **1020** |

Finally, whether there was a surface depletion of manganese due to the heat annealing treatment was identified on the different sample specimens. The results which were obtained are shown in table 8.

As may be noted, the depletion involves a layer which is no more than 4-5 microns, which may easily be removed with a common operation of abrasive brushing after the heat treatment.

From the comparison among the various materials, it may also be noted that the tested CuMn20 alloy is suitable to replace the stainless steel in any application, such as the manufacture of furniture, tools, work surfaces, etc., having a considerable hardness and high mechanical resistance, well beyond those of brasses.

### EXAMPLE 2

The antimicrobial properties of three different copper alloys were compared, and specifically the CuMn20 alloy (alloy 3) according to the invention, previously prepared according to the previous examples, a CuSn6Zn6 alloy (alloy 2) and a CuZn10 alloy (alloy 1), with two different reference materials and specifically DHP copper AISI 304 steel (stainless steel).

Three different pathogen microorganisms were used for the tests, specifically E. coli, MSRA and Listeria monocytogenes.

Flat sheet sample specimens, made of the tested alloys and of the reference materials, each of a size equivalent to about 5.5 cm² were treated with 10 microlitres of microbial cell suspension in water, having a concentration of about 108 cell units per millilitre.

Subsequently, the sample specimens were incubated at 37°C. The test was repeated 6 times, varying the time of contact in incubation. Each sample specimen was tested for the following times: 0, 5, 10, 20, 40 and 80 minutes.

After each incubation step was finished, the sample specimen was recovered and treated with an aqueous solution to remove the pathogens; the solution was then diluted and incorporated in agar and a microscopical count was finally carried out on the survived microbial cells.

The results which were obtained are shown in figures 2, 3 and 4.

As may be noted, the antimicrobial activity of the previously prepared and machined alloy, CuMn20 is substantially very similar to that of copper DHP against all of the tested pathogenic microorganisms, while stainless steel is substantially devoid thereof. The antimicrobial activity of the CuMn20 alloy is also comparable (or better), with the content of copper being the same, with respect to that of the other tested alloys, which however have a mechanical resistance and hardness that make them unsuitable to replace steel and, especially, do not have a colour comparable to that of steel, while the CuMn20 alloy according to the invention has a white metal colour comparable to that of steel.

### EXAMPLE 3

Four cylindrical ingots were prepared having a diameter of 305 mm using standard copper ingot moulds with an inner graphite insert so as to render less drastic the cooling of the metal in the ingot mould and therefore avoid the formation of contraction cracks. The metal was taken to a temperature of 1140°C in the melting furnace and, after the analytical controls to verify the adherence to the nominal composition, was poured in the holding furnace; the casting started when the metal reached the temperature of 1100 °C.

The chemical composition resulting from the mean of the two samples of cast withdrawn respectively at the beginning and at the end of each casting is shown in table 9.

**Table 9 Mean chemical composition of the cylindrical ingots in Cu80Mn20.**

| Melting N. | Cu % | Mn % | Fe % | Ni % | Sn % | Pb % |
|---|---|---|---|---|---|---|
| L88277 | 80.9 | 19.04 | 0.025 | 0.032 | <0.01 | <0.01 |
| L88278 | 79.8 | 20.10 | 0.012 | 0.028 | <0.01 | 0.01 |
| L88279 | 79.5 | 20.40 | 0.017 | 0.039 | <0.01 | 0.01 |
| L88280 | 79.7 | 20.20 | 0.020 | 0.035 | <0.01 | <0.01 |

Subsequently, the double-hole extrusion of the ingots was performed so as to obtain wires with a diameter of 26 mm, with a 4000 ton press in a range of extrusion temperatures from 770 to 800 °C, spraying the outputted wires with water coming from appropriate sprayers to limit oxidation of the alloy and/or the depletion of Mn. In these conditions the power absorbed by the press, expressed in tons, varies from 2000 to 2300 due to the high mechanical features of the Cu80Mn20 alloy. From the metallographic point of view, the best results both as regards the mean diameter of the grain and as regards the homogeneity thereof, were obtained with an extrusion temperature equivalent to 780°C. Later, the extruded products were rolled to a diameter of 20 mm and an annealing was performed for 3 hours at 650°C in a reducing atmosphere. Different cold plastic deformation (drawing) operations were then performed from a semifinished product having a 20mm-diameter to a wire having a 2.08mm-diameter, performing an intermediate step of milling from 5.70 to 5.30 mm to remove the layers of oxidation and depletion of Mn, the depth of which was less than that identified for the corresponding layers of example 1 for the rolled products. Finally, after a complete re-crystallization annealing performed at 650°C for 3 hours in a reducing atmosphere, the wires were subjected to a final step of cold drawing to a 2mm- or 1.80mm-diameter, so as to obtain a work hardening of 7.4% or, respectively, of 25% and therefore give rise, with the same alloy, to a final wire material in a medium-hard or hard physical state. As a final step, the possible brushing ensured the absence of surface layers of oxide or of layers depleted of Mn.

The values of the mechanical features which may be obtained by means of the drawing operations, depending on the different possible strain hardening, are shown in table 10.

**Table 10 Summary of the mean values of Rm, Rp and HV measured during the cold plastic deformation cycle as a function of the percentage strain hardening the Cu80Mn20 wire undergoes.**

| Strain hardening | Rm MPa | Rp MPa | HV 500g/15" |
|---|---|---|---|
| 0 | 490 | 240 | 150 |
| 7.4 | 540 | 310 | 170 |
| 25 | 717 | 450 | 195 |
| 37 | 790 | 580 | 215 |
| 55 | 827 | 710 | 235 |
| 85 | 875 | 835 | 250 |

### EXAMPLE 4

Billets of Cu80Mn20 alloy were extruded under water to tubes having a 100mm-diameter, 11mm-thickness wall, so as to limit the formation of surface oxides and/or layers depleted of Mn.

The extrusion of the billet in the form of a tube was performed in a range of extrusion temperatures in the range between 790 and 805°C. In these conditions, the power absorbed by the press, expressed in bars, was about 290, which is an acceptable value considering the high mechanical features of the Cu80Mn20 alloy.

Subsequently, a cold plastic deformation processing was performed using a pilgrim mill set at 70 hits/minute with a feed of 11.11 mm until tubes having a 45mm-diameter by a 2.25-wall thickness were obtained and later the semifinished products obtained thereby were subjected to a single operation of rectilinear cold drawing to a 35mm-diameter by 1.90 mm-thickness and a following annealing at 650°C for 4 hours in a reducing atmosphere. Subsequently, a series of coil drawing operations (to the spinners) were performed up to a 9.52mm-diameter by a 0.45mm-thickness as well as a final annealing at 650°C for 4 hours in a funnel type furnace with a reducing atmosphere. The possible final brushing ensured the absence of surface layers of oxide and/or of layers depleted of Mn.

## Claims

1. A method for producing articles, these articles being preferably intended to be employed in the health and/or food field, these articles being provided with intrinsic antibacterial properties, the method **characterised in that** it comprises the steps of:
- casting a plate or a cylindrical ingot made of a copper-based alloy containing manganese as the main alloying element, in an amount such as to make the alloy white in colour and to impart a crystalline structure in alpha phase at ambient temperature thereto, wherein said alloy contains manganese in a varying weight percentage between 15% and 40%, optionally up to 2% tin, and does not contain aluminum, and neither zinc, except as impurities, balance copper;
- subjecting the plate or ingot to a series of hot plastic deformation machining treatments in sequence, preferable rolling or drawing or extrusion, to obtain a first, predetermined percentage of sectional reduction;
- subjecting the hot semifinished article to a series of cold plastic deformation machining treatments in sequence, preferably rolling or drawing, to obtain a second, predetermined percentage of sectional reduction;
- subjecting the cold semifinished article thus obtained to one or more heat annealing treatments of complete re-crystallization, in a reducing atmosphere;
- subjecting the hot and/or cold semifinished article to at least one step of removing a surface layer thereof with a low manganese content;
- subjecting the cold, annealed, semifinished article to a step of abrasive brushing, wherein said step of abrasive brushing is performed so as to remove the surface layer of the cold, annealed, semifinished article having a thickness equal to 4 microns; and
- obtaining a desired article with the cold, annealed, semifinished article.

2. The method according to claim 1, **characterized in that** said first and second predetermined percentages of sectional reduction are on the order of 90%.

3. The method according to claim 1 or 2, **characterized in that** said step of complete re-crystallization annealing of the cold semifinished article is performed at a temperature ranging between 550°C and 750°C, in either a static or a tunnel type furnace, and in a reducing atmosphere.

4. The method according to anyone of claims from 1 to 3, **characterized in that** the hot semifinished article is subjected to a step of surface milling for removing the oxidised, low manganese layers.

## Patentansprüche

1. Verfahren zum Herstellen von Gegenständen, wobei diese Gegenstände vorzugsweise dazu bestimmt sind, im Gesundheits- und/oder Lebensmittelbereich eingesetzt zu werden, wobei diese Gegenstände mit intrinsischen antibakteriellen Eigenschaften versehen sind, **dadurch gekennzeichnet, dass** es die folgenden Schritte umfasst:
- Gießen einer Platte oder eines zylindrischen Barrens, der aus einer Legierung aus auf Kupferbasis hergestellt ist, die Mangan als das Hauptlegierungselement enthält, in einer solchen Menge, dass die Legierung eine weiße Farbe annimmt und eine kristalline Struktur in der Alpha-Phase bei Umgebungstemperatur erhält, wobei die Legierung Mangan in einem variierenden Gewichtsprozentsatz zwischen 15 % und 40 % enthält, gegebenenfalls bis zu 2 % Zinn, und kein Aluminium und auch kein Zink, außer als Verunreinigungen, als Rest Kupfer enthält;
- Unterziehen der Platte oder des Barrens einer Reihe von aufeinanderfolgenden Behandlungen der heißen plastischen Verformung in Folge, vorzugsweise Walzen oder Ziehen oder Extrudieren, um einen ersten, vorbestimmten Prozentsatz der abschnittsweisen Reduzierung zu erhalten;
- Unterziehen des heißen halbfertigen Gegenstandes einer Reihe von aufeinanderfolgenden Bearbeitungen der kalten plastischen Verformung, vorzugsweise Walzen oder Ziehen, um einen zweiten, vorbestimmten Prozentsatz der abschnittsweisen Reduzierung zu erhalten;
- Unterziehen des so erhaltenen kalten halbfertigen Gegenstandes einer oder mehreren Wärmebehandlungen einer vollständigen Rekristallisation in einer reduzierenden Atmosphäre;
- Unterziehen des heißen und/oder kalten halbfertigen Gegenstands von zumindest einem Schritt des Entfernens einer Oberflächenschicht mit einem niedrigem Mangangehalt;
- Unterziehen des kalten, geglühten, halbfertigen Gegenstands einem Schritt des Schleifbürstens, wobei der Schritt des Schleifbürstens so durchgeführt wird, dass die Oberflächenschicht des kalten, geglühten, halbfertigen Gegenstands mit einer Dicke gleich 4 Mikron entfernt wird; und
- Erhalten eines gewünschten Gegenstands mit dem kalten, geglühten, halbfertigen Gegenstand.

2. Verfahren nach Anspruch 1, **dadurch gekennzeichnet, dass** der erste und der zweite vorbestimmte Prozentsatz der abschnittsweisen Reduzierung in der Größenordnung von 90 % liegen.

3. Verfahren nach Anspruch 1 oder 2, **dadurch gekennzeichnet, dass** der Schritt des vollständigen Rekristallisationsglühens eines zeitlichen kalten halbfertige Gegenstands bei einer Temperatur zwischen 550 °C und 750 °C entweder in einem statischen oder einem tunnelartigen Ofen und in einer reduzierenden Atmosphäre durchgeführt wird.

4. Verfahren nach einem der Ansprüche von 1 bis 3, **dadurch gekennzeichnet, dass** der heiße halbfertige Gegenstand einem Schritt des Oberflächenfräsens zum Entfernen der oxidierten, manganarmen Schichten unterzogen wird.

## Revendications

1. Procédé de fabrication d'articles, ces articles étant de préférence destinés à être utilisés dans le domaine de la santé et/ou de l'alimentation, ces articles étant dotés de propriétés antibactériennes intrinsèques, le procédé étant **caractérisé en ce qu'**il comprend les étapes de :
- couler une plaque ou un barreau cylindrique constitué d'un alliage à base de cuivre contenant du manganèse en tant qu'élément d'alliage principal, en une quantité telle que l'alliage soit de couleur blanche et pour lui conférer une structure cristalline en phase alpha à température ambiante, dans lequel ledit alliage contient du manganèse dans un pourcentage de poids variant entre 15% et 40%, éventuellement jusqu'à 2%, d'étain, et ne contient pas d'aluminium, ni de zinc comme impuretés, le reste étant du cuivre ;
- soumettre la plaque ou le barreau à une série de traitements d'usinage par déformation plastique à chaud en séquence, de préférence par laminage ou étirage ou extrusion, pour obtenir un premier pourcentage prédéterminé de réduction de section ;
- soumettre l'article semi-fini chaud à une série de traitements d'usinage par déformation plastique à froid en séquence, de préférence par laminage ou étirage, pour obtenir un second pourcentage prédéterminé de réduction de section ;
- soumettre l'article semi-fini froid ainsi obtenu à un ou plusieurs traitements de recuit thermique de recristallisation complète, dans une atmosphère réductrice ;
- soumettre l'article semi-fini chaud et/ou froid à au moins une étape d'enlèvement d'une couche superficielle de celui-ci avec une faible teneur en manganèse ;
- soumettre l'article semi-fini recuit froid à une étape de brossage abrasif, dans lequel ladite étape de brossage abrasif est effectuée de manière à enlever la couche de surface de l'article semi-fini recuit froid ayant une épaisseur égale à 4 microns ; et
- obtenir un article désiré avec l'article semi-fini recuit froid.

2. Procédé selon la revendication 1, **caractérisé en ce que** lesdits premier et second pourcentages prédéterminés de réduction de section sont de l'ordre de 90%.

3. Procédé selon la revendication 1 ou 2, **caractérisé en ce que** ladite étape de recuit complet de recristallisation de l'article semi-fini froid est effectuée à une température comprise entre 550°C et 750°C, soit dans un four statique soit dans un four de type tunnel, et dans une atmosphère réductrice.

4. Procédé selon l'une quelconque des revendications 1 à 3, **caractérisé en ce que** l'article semi-fini chaud est soumis à une étape de fraisage en surface pour éliminer les couches oxydées à faible teneur en manganèse.
